

## UNITED STATES PATENT OFFICE.

SAMUEL JOSEPH INGRAM, OF SYDNEY, NEW SOUTH WALES, AUSTRALIA.

CAPSULING OF CORKED BOTTLE MOUTHS AND A COMPOSITION OF MATTER  
USABLE THEREFOR.

No Drawing.

Application filed March 22, 1921. Serial No. 454,438.

*To all whom it may concern:*

Be it known that SAMUEL JOSEPH INGRAM, a subject of the King of Great Britain and Ireland, residing at 25 City Road Darling-  
ton, Sydney, New South Wales, Australia, has invented certain new and useful Im-  
provements in the Capsuling of Corked  
Bottle Mouths and a Composition of Matter  
Usable Therefor, of which the following is a  
specification.

This invention relates to an improved method of capsuling corked bottle mouths and to a composition of matter which may be used for such capsuling. The invention is applicable principally to the capsuling of bottles containing fermented or distilled liquors such as beer or whisky, medicines, or like preparations.

The method of capsuling corked bottle mouths according to the invention consists in dipping the cork and the neck of the bottle about the cork in a liquid compound which will not melt or crack at ordinary atmospheric temperatures after it has been applied to the corked bottle mouths, so that the contents of the bottle will be sealed. After dipping the capsuled bottles are removed from the compound and allowed to stand until the capsule has dried thereon. The compound is of such nature that it may be removed from the bottle mouth by the application of hot water at a temperature say between 180° and 212° F. The capsules may be of one or more colors; if the coloring of the capsules is to be the same the corked bottle mouths to be capsuled are sealed by dipping them into a compound of one color, but if the capsules are to be more than one color they are treated with a coloring substance as is hereinafter described. The liquid capsuling compound must be capable of drying a short time after it has been applied to the bottle mouths, and must be of such character that the moulded capsule will not be brittle, and that it will be susceptible of slight expansion or contraction without cracking, to meet varying atmospheric temperature conditions.

A compound suitable as a "white" cap-  
sule for corked bottle mouths in accordance

with the invention consists of the following ingredients:—

Glauber salt.  
Sugar (cane).  
Gelatine.  
Whiting.  
Water.

55

In preparing the said compound I may take one pint of water and dissolve one to four ounces of Glauber salt therein; a quantity of sugar between one ounce and one pound is also dissolved in one pint of water. These solutions may firstly be added to each other or they may be added separately to one pound of gelatine and the latter is allowed to soak therein for a period approximately between 8 to 12 hours. One pound of whiting, which has been worked into a thick paste with water, is added to the gelatinous mixture after the latter has been heated to such consistency that it may readily run. The mixture is stirred to blend the ingredients and it is then allowed to stand for about five minutes when it will be ready for use. The heating of the gelatinous mixture may be effected by placing the vessel containing it in hot water.

60

65

70

75

The compound may also be prepared in the following manner:— One to four ounces of Glauber salt and a quantity of sugar between one ounce and one pound are mixed, to which are added 38 ounces or about 2 pints of cold water. Such mixture is stirred until the Glauber salt and the sugar have been dissolved, and the solution is added to one pound of gelatine and allowed to stand for about 8½ hours or more. If warm instead of cold water is used to dissolve the Glauber salt and sugar, the solution thereof when added to the gelatine need only be allowed to stand for about 5½ hours. The container carrying the gelatinous mixture is then placed in hot water at a temperature ranging between 180° and 212° F. until its consistency is such that it will readily run; and one pound of whiting, which has been mixed with 12 ounces of cold water (about ½ pint) to make a paste thereof, is added to the gelatinous mixture; and the whole is stirred

80

85

90

95

100

until the ingredients of the mixture are thoroughly incorporated.

5 Tripolite may be substituted for the whiting. In place of using one pound of whiting in the preparation of the compound one pound of talc and a half pound of whiting may be used.

10 If the compound is required to be colored other than "white" a coloring substance such as cochineal or a suitable aniline dye dissolved in water is added to the compound when the whiting or its substitute has been added to the gelatinous mixture and before the total mixture has been stirred to incorporate its ingredients. The proportion of 15 liquid coloring matter so used will depend on the graduation of color required. Usually about one ounce of the liquid color will be found sufficient in preparing the compound in the proportions above specified.

20 In case the coloring of the capsules is not to be uniform, that is to say, if they are required to be of more than one color, the capsules, after their addition to the bottle 25 mouths, may be dipped in a liquid coloring substance as described when two colors are required; but if more than two colors are required, the capsules may have the requisite coloring substances applied to them by a 30 brush or other means. Instead of incorporating the coloring substance with the other ingredients of the "white" compound, the capsules may be colored to requisite monochrome color by dipping them in a 35 selected liquid coloring substance.

40 If a compound having a glossy appearance is to be produced, a sufficiency of gum arabic, which is preferably dissolved in hot water, is added to and mixed with the gelatinous mixture before described. Between 2 to 4 ounces of gum arabic added to a sufficiency of water to dissolve it will be

45 found adequate for addition to the proportions of other ingredients above mentioned. Liquid gum arabic may, however, be applied separately to the sealed capsules, either by dipping them therein or otherwise suitably coating them therewith.

50 The proportions of materials herein stated are to be understood as being approximate proportions. The quantity of sugar used in the manufacture of the compound will depend on the degree of elasticity required for the capsules; the greater the quantity of sugar used in the proportions above specified, the greater will be the elasticity of the 55 capsules.

It will be understood that the consistency of the compound may be thinned by subjecting the compound to heat such as by 60 standing the container carrying the compound in hot water as before described.

What I claim as my invention and desire to secure by Letters Patent is:—

1. A liquid capsuling composition, comprising Glauber's salt, sugar, gelatine, whiting and water.

2. A liquid capsuling composition, comprising Glauber's salt, sugar, gelatine, talc, whiting and water.

3. A liquid capsuling composition, comprising one ounce of Glauber's salt, one pound of sugar, one pound of gelatine, one pound of wetted whiting, and two pints of water.

4. A liquid capsuling composition, comprising one ounce of Glauber's salt, one pound of sugar, one pound of gelatine, one pound of talc, one-half pound of wetted whiting, and two pints of water.

75 80 In testimony whereof I have affixed my signature.

SAMUEL JOSEPH INGRAM.